

1

3,783,055

**PROPELLANT CONTAINING CONJUGATED DIENE POLYMERS REACTED WITH AT LEAST 10% OF ALIPHATIC MERCAPTAN**

William B. Reynolds, Excelsior, Minn., and John E. Mahan, Bartlesville, Okla., assignors to Phillips Petroleum Company  
No Drawing. Filed June 20, 1960, Ser. No. 37,516  
Int. Cl. C06d 5/06

U.S. CL. 149—19.9

17 Claims 10

This invention relates to improved solid propellants and to their method of preparation.

Solid propellants for the propulsion of reaction engines are becoming more and more important as the rocket field develops. One type of solid propellant that has received considerable attention is a composite of organic material, which serves as fuel and binder, and a solid oxidant such as ammonium nitrate. Propellant grains are prepared from such materials by various molding techniques and the completed grain must be capable of withstanding considerable stress and shock over broad temperature ranges. Solid propellants must be able to withstand stresses at temperatures as low as  $-70^{\circ}\text{ F}$ . and it is important that the propellant grain be improved in its low temperature tensile properties, particularly elongation.

We have discovered a method of making an improved solid propellant suitable for fabrication of propellant grains. The propellant of our invention has satisfactory tensile strengths over a broad temperature range of  $-70^{\circ}\text{ F}$ . to  $+70^{\circ}\text{ F}$ . and is unexpectedly improved with respect to elongation at temperatures of  $-40$  to  $-70^{\circ}\text{ F}$ . The propellant of our invention employs a conventional oxidant and the binder is a conjugated diene polymer which has at least 10 percent of its double bonds reacted with aliphatic mercaptan. In the preparation of this propellant the aliphatic mercaptan is reacted with the conjugated diene polymer and then the polymer is cured in admixture with the oxidant.

It is an object of our invention to provide an improved solid propellant. Another object is to provide a method of improving the low temperature properties of a solid propellant which employs a conjugated diene polymer in the binder. Still another object is to provide a solid propellant which can be formed from castable liquid polymers with improved low temperature elongation. Other objects, advantages and features of our invention will be apparent to those skilled in the art from the following description and claims.

The solid propellants of our invention comprise basically an oxidant plus a rubbery binder. Generally, the oxidant is an inorganic oxidizing salt such as an alkali metal or ammonium salt of nitric or perchloric acids. Examples of suitable oxidants are ammonium perchlorate, ammonium nitrate, sodium perchlorate, potassium nitrate, and the like. By alkali metal we mean to include lithium, sodium, potassium, rubidium, and cesium. Mixtures of these oxidants are also suitable. Preferably when mixtures of the oxidizers are utilized, one of the perchlorates is in a major proportion. The oxidizer should be ground to about 1 to 200 microns average particle size and preferably to an average particle size of about 40 to 60 microns. The amount of oxidizing salt used with respect to the total base composition, i.e., oxidizer plus binder, is usually about 70 to 90 weight percent.

The binder which can be used in the propellant of the invention can broadly be any polymer of a conjugated diene wherein the conjugated diene comprises a major portion of the polymer. Such polymers can range from rubbery materials to liquids which are curable to the solid state. When the binder is a solid the propellant com-

2

position can be mixed on a roll mill or in an internal mixer such as a Banbury. The binder forms a continuous phase with the oxidizer being a discontinuous phase in the finished propellant. After mixing, any suitable technique such as extrusion, compression molding, and the like can be employed to form the propellant grain. We prefer to practice our invention with castable liquid polymers such as described in the copending application of P. S. Hudson and C. C. Bice, Ser. No. 829,462, filed July 24, 1959.

The amount of binder employed in the propellant is broadly about 5 to 40 parts by weight per 100 parts of the base propellant and preferably about 10 to 30 parts by weight. In addition to the base propellant, which comprises oxidant and binder, other materials such as one or more reinforcing agents, plasticizers, wetting agents, anti-oxidants, and the like can be used. In some instances it is desirable to use a vulcanization accelerator, a vulcanizing agent such as sulfur or an accelerator activator such as zinc oxide. Various reinforcing agents which are sometimes employed include carbon black, wood flour, lignin, and various reinforcing resins such as styrene-divinylbenzene polymer, acrylic acid-styrene-divinylbenzene polymer, and the like. Also other rubbery materials normally used as propellant binders can be admixed in minor amounts with the materials modified according to our invention in order to make up the total binder composition.

As stated above, any polymer which is formed predominantly from conjugated dienes and is liquid, semisolid or solid can be employed to form the propellant. Among the solid polymers we prefer those having a Mooney value (ML-4 at  $212^{\circ}\text{ F}$ . ) less than 100 and more preferably less than 60.

The polymer forming the binder can be a homopolymer or copolymer of conjugated dienes having from 4 to 12 carbon atoms and preferably 4 to 8 carbon atoms per molecule. Examples of suitable conjugated dienes are 1,3-butadiene, isoprene, piperylene, methylpentadiene, 2-ethyl-1,3-butadiene, phenyl-butadiene, 3,4-dimethyl-1,3-hexadiene, 4,5-diethyl-1,3-octadiene, and the like. In addition, conjugated dienes containing reactive substituents along the chain can also be employed, such as for example, halogenated dienes, such as chloroprene, fluoroprene, and the like. Of the conjugated dienes the preferred material is butadiene, with isoprene and piperylene also being especially suitable. Copolymers of these conjugated dienes with copolymerizable monomers containing a vinylidene ( $\text{CH}_2=\text{C}$ ) group can be used with the conjugated diene in a major proportion. Preferably these comonomers contain less than 20 carbon atoms per molecule. Examples of suitable comonomers are aryl-substituted olefins, such as styrene, various alkyl styrenes, paramethoxystyrene, vinyl-naphthalene, vinyltoluene, and the like; heterocyclic nitrogen-containing monomers, such as vinylcarbazole or pyridine and quinoline derivatives containing at least one vinyl or alphamethylvinyl group, such as 2-vinylpyridine, 3-vinylpyridine, 4-vinylpyridine, 3-ethyl-5-vinylpyridine, 2-methyl-5-vinylpyridine, 3,5-diethyl-4-vinylpyridine, 2-isopropenylpyridine, 2-vinylquinoline, and the like; similar mono- and di-substituted alkenyl pyridines and the like quinolines; acrylic acid esters, such as methyl acrylate, ethyl acrylate and the like; alkacrylic acid esters, such as methyl methacrylate, ethyl methacrylate, propyl methacrylate, ethyl ethacrylate, butyl methacrylate and the like; as well as other vinylidene-containing compounds such as methyl vinyl ether, vinyl chloride, vinylidene chloride, vinylfuran, vinylacetylene, acrylonitrile, and the like.

The preferred polymers which are used in our improved propellants are those which contain functional acid groups within the polymer molecule. Such polymers can be de-

scribed as including terminally reactive polymers having the formula  $QY_n$  wherein Q comprises the conjugated diene polymer of the type described above, Y is an acidic group and  $n$  is at least 1 and preferably 2 to 4. Also included within this preferred group of polymers are copolymers of a major proportion of conjugated diene with copolymerizable carboxylic acids having a maximum of 36 carbon atoms, from 1 to 5 double bonds, and 1 to 2 carboxy groups.

The polymers containing terminal acidic groups can be prepared by contacting the monomer or monomers to be polymerized with an organo alkali metal compound, preferably an organo polyalkali metal compound. The organo alkali metal compounds contain at least 1 and preferably from 2 to 4 alkali metal atoms, and those containing 2 alkali metal atoms are more often employed. As will be explained hereinafter, lithium is the preferred alkali metal.

The organo alkali metal compounds can be prepared in several ways, for example, by replacing halogens in an organic halide with alkali metals, by direct addition of alkali metals to a double bond, or by reacting an organic halide with a suitable alkali metal compound.

The organo alkali metal compound initiates the polymerization reaction, the organo radical being incorporated in the polymer chain and the alkali metal being attached terminally to at least one end of the polymer chain. When employing polyalkali metal compounds an alkali metal is attached terminally at each end of the polymer chain. The polymers in general will be linear polymers having two ends; however, polymers containing more than two ends can be prepared within the scope of the invention.

While organo compounds of the various alkali metals can be employed in carrying out the polymerization, by far the best results are obtained with organolithium compounds which give very high conversions to the terminally reactive polymer. With organo compounds of the other alkali metals, the amount of monoterminally reactive polymer, that is, polymer having alkali metal at only one end of the chain is substantially higher. The alkali metals, of course, include sodium, potassium, lithium, rubidium, and cesium. The organic radical of the organo alkali metal compound can be an aliphatic, cycloaliphatic or aromatic radical. For example, mono-, di- and poly-alkali metal substituted hydrocarbons can be employed including

methylolithium,  
n-butyllithium,  
n-decyllithium,  
phenyllithium,  
naphthyllithium,  
p-tollyllithium,  
cyclohexyllithium,  
4-butylphenylsodium,  
4-cyclohexylbutylpotassium,  
isopropylrubidium,  
4-phenylbutylcesium,  
1,4-dilithiobutane,  
1,5-dipotassiumpentane,  
1,4-disodio-2-methylbutane,  
1,6-dilithiohexane,  
1,10-dilithiodescane,  
1,15-dipotassiumpentadecane,  
1,20-dilithioeicosane,  
1,4-disodio-2-butene,  
1,4-dilithio-2-methyl-2-butene,  
1,4-dilithio-2-butene,  
1,4-dipotassium-2-butene,  
dilithionaphthalene,  
disodionaphthalene,  
4,4'-dilithiobiphenyl,  
disodiophenanthrene,  
dilithioanthracene,  
1,2-dilithio-1,1-diphenylethane,  
1,2-disodio-1,2,3-triphenylpropane,

1,2-dilithio-1,2-diphenylethane,  
1,2-dipotassiumtriphenylethane,  
1,2-dilithiotetraphenylethane,  
1,2-dilithio-1-phenyl-1-naphthylethane,  
1,2-dilithio-1,2-dinaphthylethane,  
1,2-disodio-1,1-diphenyl-2-naphthylethane,  
1,2-dilithiotrinaphthylethane,  
1,4-dilithiocyclohexane,  
2,4-disodioethylcyclohexane,  
3,5-dipotassium-n-butylcyclohexane,  
1,3,5-trilithiocyclohexane,  
1-lithio-4-(2-lithiomethylphenyl)butane,  
1,2-dipotassium-3-phenylpropane,  
1,2-di(lithiobutyl)benzene,  
1,3-dilithio-4-ethylbenzene,  
1,4-dirubidiobutane,  
1,8-dicesiooctane,  
1,5,12-trilithiododecane,  
1,4,7-trisodioheptane,  
1,4-di(1,2-dilithio-2-phenylethyl)benzene,  
1,2,7,8-tetrasodionaphthalene,  
1,4,7,10-tetrapotassiumdecane,  
1,5-dilithio-3-pentyne,  
1,8-disodio-5-octyne,  
1,7-dipotassium-4-heptyne,  
1,10-dicesio-4-decyne, and  
1,11-dirubidio-5-hendecyne,  
1,2-disodio-1,2-diphenylethane,  
dilithiophenanthrene,  
1,2-dilithiotriphenylethane,  
1,2-disodio-1,1-diphenylethane,  
dilithiomethane,  
1,4-dilithio-1,1,4,4-tetraphenylbutane,  
1,4-dilithio-1,4-dinaphthylbutane,  
and the like.

While the organo alkali metal initiators in general can be employed, certain specific initiators give better results than others and are preferred in carrying out the preparation of the terminally reactive polymers. For example, of the condensed ring aromatic compounds the lithium-anthracene adduct is preferred, but the adducts of lithium with naphthalene and biphenyl can be employed with good results. Of the compounds of alkali metals with polyaryl-substituted ethylenes, the preferred material is 1,2-dilithio-1,2-diphenylethane (lithium-stilbene adduct).

Ordinarily the dilithio compounds are preferred as being more effective in promoting the formation of terminally reactive polymers. The polymers thus formed are especially well suited for use in our invention as binders for castable rocket propellant mixtures since such materials can be cured from the liquid state to rubbery solids. The organo dialkali metal compounds which have been set forth as being preferred, are those which when prepared contain a minimum of the monoalkali metal compound.

The amount of initiator which can be used will vary depending on the polymer prepared, and particularly the molecular weight desired. Usually the terminally reactive polymers which are liquids have molecular weights in the range of 1000 to about 20,000. Depending upon the monomers employed and the amount of initiator used, semi-solid and solid terminally reactive polymers can be prepared. Usually the initiator is used in amounts between about 0.25 and about 100 millimoles per 100 grams of monomer.

Preparation of the polymers containing terminal alkali metal atoms is generally carried out in the range of between  $-100$  and  $+150^{\circ}\text{C}$ ., preferably between  $-75$  and  $+75^{\circ}\text{C}$ . The particular temperatures employed will depend on both the monomers and the initiators used in preparing the polymers. For example, it has been found that the organolithium initiators provide more favorable results at elevated temperatures whereas lower temperatures are required to effectively initiate polymerization to the desired products with the other alkali metal com-

pounds. The amount of initiator employed can vary but is preferably in the range of between about 1 and about 30 millimoles per 100 grams of monomers. It is preferred that the polymerization be carried out in the presence of a suitable diluent, such as benzene, toluene, cyclohexane, methyl cyclohexane, xylene, n-butane, n-hexane, n-heptane, isooctane, and the like. Generally, the diluent is selected from hydrocarbons, e.g., paraffins, cycloparaffins, and aromatics containing from 4 to 10 carbon atoms per molecule. As stated previously, the organodilithium compounds are preferred as initiators in the polymerization reaction since a very large percentage of the polymer molecules formed contain two terminal reactive groups, and also the polymerization can be carried out at normal room temperatures. This is not to say, however, that other organo alkali metal initiators cannot be employed; however, usually more specialized operation or treatment is required with these materials, including low reaction temperatures. Since it is desirable to obtain a maximum yield of terminally reactive polymer, it is within the scope of the invention to use separation procedures, particularly with alkali metal initiators other than lithium compounds, to separate terminally reactive polymer from the polymer product.

The terminally reactive polymers prepared as hereinbefore set forth contain an alkali metal atom on at least one end and preferably on each end of the polymer chain and the organic radical of the initiator is present in the polymer chain. These terminally reactive polymers when treated with suitable reagents such as carbon dioxide, sulfonyl chloride, etc., and hydrolyzed provide polymers containing terminal acid groups. The acidic groups include groups such as SOH, SO<sub>2</sub>H, SO<sub>3</sub>H, COOH, SeO<sub>2</sub>H, SeO<sub>3</sub>H, SiO<sub>2</sub>T, SnO<sub>2</sub>H, SbO<sub>2</sub>H, SbOH, SbO<sub>3</sub>H<sub>2</sub>, TeO<sub>2</sub>H, TeO<sub>3</sub>H, AsO<sub>2</sub>H, AsOH, AsO<sub>3</sub>H<sub>2</sub>, AsO<sub>3</sub>H<sub>3</sub>. The following reactions present examples of specific methods which can be employed to introduce the terminal acid groups. In these equations Q designates a polymer chain.

- (1)  $\text{Li}-\text{Q}-\text{Li} + 2\text{CO}_2 \rightarrow \text{LiCO}_2-\text{Q}-\text{CO}_2\text{Li}$   
 $\text{Li}-\text{CO}_2-\text{Q}-\text{CO}_2\text{Li} + 2\text{HCl} \rightarrow \text{HOOC}-\text{Q}-\text{COOH} + 2\text{LiCl}$
- (2)  $\text{Li}-\text{Q}-\text{Li} + \text{SO}_2\text{Cl}_2 \rightarrow \text{LiSO}_2\text{Cl}_2-\text{Q}-\text{SO}_2\text{Cl}_2\text{Li}$   
 $\text{LiSO}_2\text{Cl}_2-\text{Q}-\text{SO}_2\text{Cl}_2\text{Li} + 2\text{H}_2\text{O} \rightarrow \text{HO}_3\text{S}-\text{Q}-\text{SO}_3\text{H} + 2\text{LiCl} + 2\text{HCl}$

Reaction of terminally reactive polymer containing alkali metal atoms with the acid forming reagents can be carried out over a wide range of temperatures, for example -75° C. to +75° C., and preferably utilizing an amount of reagent in excess of stoichiometric.

The monomers hereinbefore described for use in preparation of terminal reactive polymers containing alkali metal atoms can also be reacted with unsaturated carboxylic acids to provide liquid polymers suitable for use in carrying out the invention. Unsaturated carboxylic acids which can be employed include acids containing up to 36 carbon atoms, from 1 to 5 double bonds and 1 or 2 carboxyl groups. Also included are the so-called "dimerized" acids, i.e. where two molecules of an acid are linked by destroying one of the double bonds. Illustrative of specific acids which can be used are acids such as acrylic acid, methacrylic acid, itaconic acid, palmitoleic acid, oleic acid, ricinoleic acid, arachidonic acid, erucic acid, selacholeic acid, fumaric acid, maleic acid, and the like. Reaction of the monomer with the unsaturated carboxylic acid can be carried out over a wide range of temperatures depending on the particular monomer and the particular acid employed; e.g. at temperatures between about -50 and about +100° C. The amount of acid employed in the reaction can vary to provide polymers having an acid equivalence of from as low as 0.005 to as high as 0.2 equivalent per 100 grams of polymer product.

While the polymers containing the terminal acidic groups are preferred for the practice of the invention, polymers containing other terminally reactive groups such as hydroxy groups or mercapto groups can be employed. Such polymers and their preparation and curing as well as other types of terminally reactive polymers which can be used in our invention are described in the copending application of Carl A. Uranek et al., Ser. No. 772,167, filed Nov. 6, 1958. The liquid polymers thus formed are mixed with the oxidant and cured to solid rubbery compositions. The polymers containing carboxy groups in the molecule can be cured with epoxides, tri(aziridinyl)phosphine oxides or sulfides. These agents can be represented by the formula



wherein X is selected from the group consisting of oxygen and sulfur, P is phosphorus, the R's are radicals containing up to a total of 20 carbon atoms selected from the group consisting of hydrogen, alkyl, cycloalkyl, aryl, alkaryl, and aralkyl radicals and the R's can be unlike. Specific phosphine reactants which can be used include

- 30 tri(1-aziridinyl)phosphine oxide,
- 31 tri(2-methyl-1-aziridinyl)phosphine oxide,
- 32 tri(2,3-dimethyl-1-aziridinyl)phosphine oxide,
- 33 tri(2-isopropyl-1-aziridinyl)phosphine oxide,
- 34 tri(2-methyl-3-ethyl-1-aziridinyl)phosphine oxide,
- 35 tri(2-isopropyl-1-aziridinyl)phosphine oxide,
- 36 tri(2-methyl-3-n-butyl-1-aziridinyl)phosphine oxide,
- 37 tri(2-hexyl-1-aziridinyl)phosphine oxide,
- 38 tri(2,3-diheptyl-1-aziridinyl)phosphine oxide,
- 39 tri(2-methyl-3-octyl-1-aziridinyl)phosphine oxide,
- 40 tri(2-ethyl-3-decyl-1-aziridinyl)phosphine oxide,
- 41 tri(2-dodecyl-1-aziridinyl)phosphine oxide,
- 42 tri(2-methyl-3-tridecyl-1-aziridinyl)phosphine oxide,
- 43 tri(2-ethyl-3-octadecyl-1-aziridinyl)phosphine oxide,
- 44 tri(2-eicosyl-1-aziridinyl)phosphine oxide,
- 45 tri(2-methyl-3-cyclopentyl-1-aziridinyl)phosphine oxide,
- 46 tri(2-ethyl-3-cyclohexyl-1-aziridinyl)phosphine oxide,
- 47 tri[2-n-butyl-3-(4-methylcyclohexyl)1-aziridinyl]phosphine oxide,
- 48 tri(2-phenyl-1-aziridinyl)phosphine oxide,
- 49 tri(2-phenyl-3-tetradecyl-1-aziridinyl)phosphine oxide,
- 50 tri(2,3-diphenyl-1-aziridinyl)phosphine oxide,
- 51 tri(2-tert-butyl-3-phenyl-1-aziridinyl)phosphine oxide,
- 52 tri[2-ethyl-3-(1-naphthyl)1-aziridinyl]phosphine oxide,
- 53 tri[2-n-propyl-3-(2-naphthyl)1-aziridinyl]phosphine oxide,
- 54 tri(2-methyl-3-benzyl-1-aziridinyl)phosphine oxide,
- 55 tri(2-nonyl-3-benzyl-1-aziridinyl)phosphine oxide,
- 56 tri[2-n-propyl-3-(2-phenylethyl)1-aziridinyl]phosphine oxide,
- 57 tri[2-methyl-3-(4-methylphenyl)1-aziridinyl]phosphine oxide,
- 58 tri[2-ethyl-3-(3-n-propylphenyl-1-aziridinyl)phosphine oxide,
- 59 tri[2-heptyl-3-(2,4-dimethylphenyl)1-aziridinyl]phosphine oxide,
- 60 tri(1-aziridinyl)phosphine sulfide,
- 61 tri(2-methyl-1-aziridinyl)phosphine sulfide,
- 62 tri(2,3-dimethyl-1-aziridinyl)phosphine sulfide,
- 63 tri(2,3-diethyl-1-aziridinyl)phosphine sulfide,
- 64 tri(2-methyl-3-isopropyl-1-aziridinyl)phosphine sulfide,
- 65 tri(2-tert-butyl-1-aziridinyl)phosphine sulfide,
- 66 tri(2,3-didecyl-1-aziridinyl)phosphine sulfide,
- 67 tri(2-ethyl-3-pentadecyl-1-aziridinyl)phosphine sulfide,
- 68 tri(2-eicosyl-1-aziridinyl)phosphine sulfide,
- 69 tri(2-methyl-3-cyclohexyl-1-aziridinyl)phosphine sulfide,
- 70 tri(2-phenyl-1-aziridinyl)phosphine sulfide,

tri(2-phenyl-3-benzyl-1-aziridinyl)phosphine sulfide, tri(2,3-diphenyl-1-aziridinyl)phosphine sulfide, tri(2-ethyl-3-phenyl-1-aziridinyl)phosphine sulfide, and tri(2-amyl-3-benzyl-1-aziridinyl)phosphine sulfide.

Suitable epoxide curatives are various commercially available epoxide resins, for example, Bisphenol A which has the general formula:



or Shell Epon X-701 having the general formula:



Polymers containing terminal hydroxy or mercapto groups can be cured with isocyanates. The polymers containing terminal mercapto groups can also be cured with heat alone or with diphenyl dioxime plus magnesium oxide.

In order to improve the low temperature properties of the solid propellant the polymer is reacted prior to curing with an aliphatic mercaptan containing from 1 to 16 carbon atoms. Preferably aliphatic mercaptans containing from 2 to 8 carbon atoms are used. Examples of suitable mercaptans are methyl mercaptan, ethyl mercaptan, isopropyl mercaptan, butyl mercaptan, 2-methyl-3-mercaptopentane, 1-mercaptop-m-octane, 2-mercaptop-2,3-dimethyl heptane, 2-mercaptop-2,4-dimethyl octane, tert-pentyl mercaptan, secondary dodecyl mercaptan, 2-mercaptop-3,4-diethyl decane, 3-mercaptop-2-propyl-4-methyl dodecane and the like.

The reaction between the polymer and the mercaptan can be readily effected by merely mixing the polymer and mercaptan together, generally with a substantial excess of mercaptan. Irradiating the mixture with ultraviolet light hastens the reaction. The reaction should be continued until at least 10 percent of the double bonds of the polymer molecules are reacted with the mercaptan. When the polymers in which functional groups are present at the ends or along the polymer molecule the reaction with the mercaptan can be carried out until substantially all of the double bonds have reacted. Among the other polymers where curing is effected across double bonds the reaction with the mercaptan should not exceed about 80 percent of the double bonds available. The polymers thus reacted with the aliphatic mercaptans can be mixed with the oxidant and cured to form the propellant grain. If desired, the mercaptan can be reacted with the polymer in the presence of the oxidant with the curing agent added subsequently.

When preparing the preferred propellants of the invention employing the polymers containing functional acidic groups within the molecule, the polymers are admixed with the tri(aziridinyl)phosphine oxide or sulfide and the inorganic oxidizing salt, after which the mixture is suitably increased in temperature such that reaction occurs between the polymer and the phosphine compound to provide a solid propellant structure. In the preparation of the binder from liquid polymer the polymer and phosphine reactant are placed in a suitable dispersant-type mixer and thoroughly mixed for a period of 1 to 10 minutes. The oxidizer which is finely powdered to a size in the range of from about 20 to 200 microns is then added and mixing

is continued for a period of 15 to 45 minutes under vacuum. During the latter mixing step the temperature is gradually increased to a temperature between about 100 to 300° F., preferably between about 150 and about 200° F. The material at this stage is a viscous slush, which is then poured into a rocket case or suitable mold. The filled mold is placed in an oven and cured for 24 to 48 hours or more at temperatures in the range of 150 to 200° F. Semi-solid polymers can be blended with the phosphine reactant and oxidizer and the mixture extruded to form a curable propellant grain.

In addition to the binder and the oxidant, the propellants of this invention can contain a powdered metal or a metal halide. Suitable metals are aluminum, boron, magnesium beryllium, and the like. Alloys such as aluminum alloys of boron, magnesium, manganese, copper, and the like can also be used. Silicon can be utilized and the term "metal" is used herein to include silicon. In the propellant composition the metal can replace part of the oxidant and the solids (oxidizer plus metal) loading can vary from 70 to 85 weight percent of the base with 15 to 30 percent binder. The oxidizer should be 70 to 100 percent of the solids with 0 to 30 percent as the metal. Generally the components of the solid propellant compositions of this invention are present in the relative amounts set forth below.

| Component:               | Weight percent |
|--------------------------|----------------|
| Inorganic oxidizing salt | 75-85          |
| Acidic polymer           | 15-25          |
| Powdered metal           | 0-10           |

In addition to other additives, burning rate catalysts can be incorporated into the propellant composition. These catalysts include materials such as ferrocyanides sold under various trade names, such as Prussian blue, Steel blue, Bronze blue, Turnbull's blue, Chinese blue, New blue, Antwerp blue, Mineral blue, Paris blue, Berlin blue, Hamburg blue, Williamson blue, and the like. Other useful burning rate catalysts include copper chromite, ammonium dichromate, potassium dichromate, sodium dichromate, and the like.

To further illustrate our invention the following examples are presented giving conditions which should be considered as typical and not limit our invention unduly.

#### EXAMPLE I

Polybutadiene having terminal carboxy groups and the following properties was treated with n-butyl mercaptan in solution under the influence of ultraviolet radiation. The polymer had a viscosity of 1500 poises, a carboxy content of 1.82 percent and a vinyl content of about 50 percent. It had been prepared in cyclohexane solvent with 40 millimoles of lithium stilbene adduct employed as the initiator.

In reacting the polymer with the mercaptan 75 grams of polymer were dissolved in 306 grams of n-butyl mercaptan and the solution was irradiated one hour with the light from a 100 watt mercury vapor lamp. Based on the weight increase of the recovered polymer and assuming 90 percent unsaturation, about 50 percent of the double bonds had reacted with the mercaptan.

The mercaptan-treated polybutadiene containing terminal carboxy groups was mixed with ammonium perchlorate and cured with tri(2-methyl-1-aziridinyl)phosphine oxide to form Propellant A. As a control the same polymer which had not been reacted with the mercaptan was mixed with ammonium perchlorate and cured with the tri(aziridinyl)phosphine oxide to form Propellant B. The recipes were as follows.

| Propellant A:                                           | Weight percent |
|---------------------------------------------------------|----------------|
| Carboxy-containing polybutadiene, 50% n-butyl mercaptan | 19.65          |
| Tri(aziridinyl)phosphine oxide                          | 0.35           |
| Ammonium perchlorate                                    | 80.00          |

| Propellant B:                    | Weight percent |
|----------------------------------|----------------|
| Carboxy-containing polybutadiene | 19.37          |
| Tri(aziridinyl)phosphine oxide   | 0.63           |
| Ammonium perchlorate             | 80.00          |

The amount of curative used was on an equivalent basis of  $-\text{COOH}$  in the polymer. This goes down as the molecular weight increases as a result of the addition of mercaptan.

After curing for 96 hours at  $160^{\circ}\text{ F}$ . the propellant compositions were evaluated for tensile strengths at low temperatures. The results are shown in Table I.

TABLE I

| Propellant | T, $^{\circ}\text{ F}$ . | P.s.i. |       | Percent <sup>1</sup> |              |
|------------|--------------------------|--------|-------|----------------------|--------------|
|            |                          | $S_m$  | $S_b$ | $\epsilon_m$         | $\epsilon_b$ |
| A          | -40                      | 478    | 418   | 22.2                 | 49.1         |
| B          | -40                      | 681    | 618   | 11.0                 | 17.3         |
| A          | -70                      | 1,405  | 1,196 | 1.7                  | 3.6          |
| B          | -70                      | 2,123  | ----- | 0.9                  | 98,300       |
|            |                          |        |       |                      | 217,000      |

<sup>1</sup> See "Method for Determining the Tensile Properties of Solid Rocket Propellants," Part II, Solid Propellant Information Agency, Johns Hopkins University, Silver Spring, Maryland, February 1957.

NOTE.— $S_m$  = maximum tensile strength;  $S_b$  = tensile strength at break,  $\epsilon_m$  = elongation at maximum stress;  $\epsilon_b$  = elongation at break; E = Young's modulus.

These data show that the addition of butyl mercaptan doubled the elongation at  $-40^{\circ}\text{ F}$ . and the modulus was reduced by one-half at  $-70^{\circ}\text{ F}$ . In addition, the propellant made with the butyl mercaptan treated polymer gave a typical stress-strain curve for rubbery materials at  $-70^{\circ}\text{ F}$ . The control propellant did not show this rubbery type of stress-strain behavior.

## EXAMPLE II

The same polymer employed in Example I was reacted with butyl mercaptan until about 5 percent of the double bonds were reacted. This polymer was mixed with ammonium perchlorate and cured as in Example I with the tri(aziridinyl)phosphine oxide according to the following recipe.

| Weight percent                                        |       |
|-------------------------------------------------------|-------|
| Carboxy-containing polybutadiene, 15% butyl mercaptan | 19.47 |
| Tri(aziridinyl)phosphine oxide                        | .53   |
| Ammonium perchlorate                                  | 80.00 |

The polymer was cured for 96 hours at  $160^{\circ}\text{ F}$ . The tensile properties of the cured propellant are shown in Table II.

TABLE II

| T, $^{\circ}\text{ F}$ . | P.s.i. |       | Percent      |              | E, p.s.i. |
|--------------------------|--------|-------|--------------|--------------|-----------|
|                          | $S_m$  | $S_b$ | $\epsilon_m$ | $\epsilon_b$ |           |
| -40                      | 555    | 448   | 14.2         | 21.8         | 7,260     |
| -70                      | 1,672  | ----- | 1.1          | -----        | 159,000   |

Even with only 15 percent of the double bonds reacted with mercaptan there is a definite improvement in low temperature properties over the control Propellant B of Table I.

As will be evident to those skilled in the art, various modifications of this invention can be made, or followed, in the light of the foregoing disclosure and discussion, without departing from the spirit or scope thereof.

We claim:

1. An improved solid propellant comprising inorganic oxidizing salt and binder which is predominantly a cured rubbery polymer containing a major amount of combined conjugated diene having 4 to 12 carbon atoms, said polymer before curing having at least 10 percent of its double bonds reacted with aliphatic mercaptan of from 1 to 16 carbon atoms.

2. An improved solid propellant comprising, per 100 parts of propellant, from 70 to 85 parts by weight of oxidant selected from the group consisting of alkali metal and ammonium salts of nitric and perchloric acids and

mixtures thereof and 15 to 30 parts by weight binder which is predominantly a cured rubbery polymer containing a major amount of combined conjugated diene having 4 to 12 carbon atoms, said polymer before curing having at least 10 percent of its double bonds reacted with aliphatic mercaptan of from 1 to 16 carbon atoms.

3. The propellant of claim 2 wherein said polymer contains at least one carboxyl group per molecule.

4. The propellant of claim 3 wherein said polymer has been cured by reaction with a polyfunctional aziridinyl phosphine compound.

5. An improved solid propellant comprising about 70 to 90 weight percent inorganic oxidizing salt and about 10 to 30 weight percent binder which is predominantly a polymer formed by reacting an aliphatic mercaptan of 1 to 16 carbon atoms with at least 10 percent of the double bonds of a conjugated diene polymer selected from the group consisting of homopolymers of conjugated dienes having 4 to 12 carbon atoms and copolymers of a major proportion of said conjugated dienes with copolymerizable vinylidene-containing monomers, said polymer containing at least 1 acidic group per molecule, and subsequently cured in admixture with said oxidizing salt with a reactant material having the formula



wherein X is selected from the group consisting of oxygen and sulfur, P is phosphorus, the R's are radicals containing up to a total of 20 carbon atoms selected from the group consisting of hydrogen, alkyl, cycloalkyl, aryl, alkaryl, and aryl radicals, and the R's can be unlike.

6. The propellant of claim 5 wherein said conjugated diene polymer is a liquid polymer having the formula  $QY_n$  wherein Q comprises a polymer of vinylidene-containing monomers, Y is a terminal acidic group and n is an integer of 1 to 4.

7. The propellant of claim 5 wherein said conjugated diene polymer is a copolymer of vinylidene-containing monomers with unsaturated carboxylic acids having a maximum of 36 carbon atoms, from 1 to 5 double bonds and from 1 to 2 carboxyl groups.

8. An improved solid propellant comprising about 70 to 85 weight percent inorganic oxidizing salt and 15 to 30 weight percent binder which before curing is a liquid polymer of butadiene, said polymer containing terminal carboxy groups with at least 10 percent of the double bonds of said polymer reacted with aliphatic mercaptans of 2 to 8 carbon atoms, and said polymer having been cured by reaction with a reactant material having the formula



wherein X is selected from the group consisting of oxygen and sulfur, P is phosphorus, the R's are radicals containing up to a total of 20 carbon atoms selected from the group consisting of hydrogen, alkyl, cycloalkyl, aryl, alkaryl, and aryl radicals, and the R's can be unlike.

9. The propellant of claim 8 wherein said reactant material is tri(aziridinyl)phosphine oxide.

10. An improved solid propellant comprising about 70 to 85 weight percent inorganic oxidizing salt and 15 to 30 weight percent binder which is a copolymer of butadiene in major amount and acrylic acid with at least 10 percent of the double bonds of said polymer reacted with aliphatic mercaptans of 2 to 8 carbon atoms, and said

polymer having been cured by reaction with a reactant material having the formula



wherein X is selected from the group consisting of oxygen and sulfur, P is phosphorus, the R's are radicals containing up to a total of 20 carbon atoms selected from the group consisting of hydrogen, alkyl, cycloalkyl, aryl, alkaryl, and aryl radicals, and the R's can be unlike.

11. An improved solid propellant comprising 70 to 85 weight percent ammonium perchlorate and 15 to 30 weight percent butadiene polymer having terminal carboxyl groups and at least 20 percent of its double bonds reacted with butyl mercaptan and cured with tri(aziridinyl) phosphine oxide.

12. A method of forming a solid propellant composition having improved low temperature properties which comprises reacting an aliphatic mercaptan of 1 to 16 carbon atoms with at least 10 percent of the double bonds of an saturated polymer containing a major amount of combined conjugated diene having 4 to 12 carbon atoms per molecule, mixing the reaction product with inorganic oxidizing salt and curing the resulting mixture.

13. A method of forming a solid propellant composition having improved low temperature properties which comprises reacting an aliphatic mercaptan of 1 to 16 carbon atoms with at least 10 percent of the double bonds of an unsaturated polymer containing a major amount of combined conjugated diene having 4 to 12 carbon atoms per molecule, said polymer containing at least one carboxyl group per molecule, mixing 15 to 30 parts by weight of the resulting polymer with 70 to 85 parts by weight of oxidant selected from the group consisting of alkali metal and ammonium salts of nitric and perchloric acids and mixtures thereof, and curing the resulting mixture by reacting said polymer with a polyfunctional(aziridinyl)phosphine compound.

14. A method of forming a solid propellant composition having improved low temperature properties which comprises reacting an aliphatic mercaptan of 1 to 16 carbon atoms with at least 10 percent of the double bonds of a conjugated diene polymer selected from the group consisting of homopolymers of conjugated dienes having 4 to 12 carbon atoms and copolymers of a major pro-

portion of said conjugated dienes with copolymerizable vinylidene-containing monomers, said polymer containing at least 1 acidic group per molecule, mixing about 10 to 30 parts by weight of the polymer-mercaptan reaction product with about 70 to 90 parts by weight of inorganic oxidizing salt, and curing the resulting mixture by reacting said polymer with a reactant material having the formula



10

15

wherein X is selected from the group consisting of oxygen and sulfur, P is phosphorus, the R's are radicals containing up to a total of 20 carbon atoms selected from the group consisting of hydrogen, alkyl, cycloalkyl, aryl, alkaryl, and aryl radicals, and the R's can be unlike.

15. The method of claim 14 wherein said conjugated diene polymer is a liquid polymer having the formula QY<sub>n</sub> wherein Q comprises a polymer of vinylidene-containing monomers, Y is a terminal acidic group and n is an integer of 1 to 4.

16. The method of claim 14 wherein said conjugated diene polymer is a copolymer of vinylidene-containing monomers with unsaturated carboxylic acids having a maximum of 36 carbon atoms, from 1 to 5 double bonds and from 1 to 2 carboxyl groups.

17. A method of forming a solid propellant composition having improved low temperature properties which comprises reacting butyl mercaptan with at least 20 percent of the double bonds of butadiene polymer having terminal carboxyl groups, and curing 15 to 30 parts by weight of the resulting polymer in admixture with 70 to 85 parts by weight of ammonium perchlorate by reaction with tri(aziridinyl) phosphine oxide.

40

#### References Cited

##### UNITED STATES PATENTS

|           |        |       |        |
|-----------|--------|-------|--------|
| 2,931,437 | 4/1960 | Smith | 149—19 |
| 2,877,504 | 3/1959 | Fox   | 149—19 |

45 BENJAMIN R. PADGETT, Primary Examiner

U.S. Cl. X.R.

149—20, 22

UNITED STATES PATENT OFFICE

CERTIFICATE OF CORRECTION

Patent No. 3,783,055      William B. Reynolds et al.      Dated January 1,

It is certified that error appears in the above-identified patent and that said Letters Patent are hereby corrected as shown below:

Column 11, line 25, "an saturated" should read --- an unsaturated ---.

Signed and sealed this 23rd day of April 1974.

(SEAL)

Attest:

EDWARD M.FLETCHER,JR.  
Attesting Officer

C. MARSHALL DANN  
Commissioner of Patents